

1

2,832,704

COATED PYROTECHNIC METAL POWDERS AND  
METHOD OF THEIR PREPARATION

Raymond H. Comyn, Silver Spring, Md.

No Drawing. Application July 1, 1952  
Serial No. 296,769

3 Claims. (Cl. 148—6.2)

(Granted under Title 35, U. S. Code (1952), sec. 266)

The invention described herein may be manufactured and used by or for the government of the United States of America for governmental purposes without the payment of any royalties thereon or therefor.

This application is a continuation-in-part of application Serial No. 213,661, filed March 2, 1951, now abandoned.

This invention relates to protective coatings for metal powders for protecting the powders against deterioration and more particularly to a process for applying a thin coating of water and chemical impervious substance to the surfaces of such powders.

Methods heretofore employed for protecting metal powders against deterioration have not proved to be entirely satisfactory for the reasons that such coating only protected the powders against deterioration for a short or limited period of time and the thickness of the coating could not be closely controlled. Furthermore, such a coating would flake off and thus expose the metal surfaces to oxidation.

Accordingly, it is an object of the present invention to provide a new and improved protective coating of controlled thickness for metal powders which will prevent deterioration of the powder.

Another object of the invention is to provide a coating for metal powders which will prevent other chemicals lying in close proximity thereto from reacting with the metal powders.

Still another object of the invention is to provide a method of producing a thin coating of water and chemical impervious substance to the surface of each particle of the metal powders for preventing deterioration and reaction thereof with other chemicals.

A further object of the invention is to provide a new and improved method of producing a thin coating of water repellent material on metallic powders which will not affect the subsequent use of the powder and which is reproducible so that the properties of the powders may be reproducible.

Other objects and many of the attendant advantages of this invention will be readily appreciated as the same becomes better understood by reference to the following detailed description.

It is well known that metal powders such, for example, as cobalt, manganese and the like are employed extensively in compounding pyrotechnic mixtures, particularly gasless delay mixtures for use in ordnance devices such, for example, as shells, rockets and the like.

Such metals as heretofore mentioned are commonly known in the trade as metal fuels and are used in pyrotechnic mixtures for causing proper delay and uniform burning time of the mixture when the mixture has been ignited. Furthermore, it is well known that the aforesaid fuels are readily affected by atmospheric conditions such, for example, as high humidity and temperature and thus causing erratic burning of the pyrotechnic in which such fuels are used.

The purpose of the present invention is to improve

2

the moisture-resistance characteristic of metal powders by coating the powders with a thin layer of water-repellent chemical of controlled thickness whereupon the properties of the powders are reproducible and thus subsequent use thereof is not affected, the powder also being protected against deterioration thereby increasing the life thereof and making the powders admirably suited for use in pyrotechnic mixtures are employed extensively in ordnance devices. Furthermore, it has been found that ordnance devices employing mixtures having the new and improved metal powders therein are extremely stable and thus can be stored over a long period of time without appreciable deterioration of the mixture due to adverse atmospheric conditions.

It is well known in the art of metal powders that moisture accelerates the deterioration thereof, such deterioration resulting from atmospheric conditions such, for example, as high humidity and temperature. In view of these unfavorable conditions existing in prior art metallic powders, the instant invention overcomes such conditions by producing chemically treated metal powders having the desirable characteristics such, for example, as being free from hydrate formation, and not subjected to decomposition in water.

The preferred process for forming a protective coating on metallic powders to make them less affected by atmospheric conditions consists of first stirring a quantity of the metal powder in a warm aqueous solution of a soluble dichromate as for example, sodium or potassium dichromate. It has been determined that a 5% solution of the dichromate at a temperature between 70 and 95° C. may be used to treat the metal powder. The metal powder is permitted to remain in the dichromate solution for a period of time approximately thirty minutes and is thereafter filtered in any suitable manner, washed with distilled water and dried. The result of this treatment is to leave a film on the powder which provides protection against atmospheric corrosion and conditions the powder for the application thereto of stearic acid. The above treatment results in an increase in the weight of the powdered metal. In one particular case, a weight increase of about 5% was noted after manganese powder was treated with a soluble dichromate and then dried, thus suggesting that the metal powder has reacted with the dichromate solution, probably forming an oxide coating on the powder.

The dried dichromate treated powder is then treated with stearic acid by stirring the dry powder in a solution of stearic acid and a suitable solvent such, for example, as ethyl ether or carbon tetrachloride for a predetermined period of time. Any desired concentration may be used and the time is not critical. When this operation has been completed the powder is again filtered and washed with a solvent similar to the aforementioned type thereby to remove excess stearic acid therefrom.

The aforesaid treatment of the powder results in uniformly coating the metal particles thereof with a thin stearic acid outer layer of water repellent material substantially a molecule thick over the film resulting from the dichromate treatment thereby to protect the powder against oxidation whereupon deterioration of the powder due to adverse atmospheric conditions is greatly reduced.

It has been found by actual tests that neither a dichromate treatment nor a stearic acid treatment alone affords the desired protection for the powder against deterioration while on the other hand it has been found that the improved method of treatment as heretofore set forth produces the desired result. For example, during these tests a powder such, for example, as manganese was employed and treated in the above mentioned manner and in each instance the treated powder was exposed

to relatively high humidity of 95% and temperature of 71° C. A test on untreated powder under the aforesaid conditions was also made. However, during such tests the treated and untreated powders were dried at predetermined intervals and weighed. Thereafter the relative deterioration was measured by percent weight increase.

The results of these tests are shown on the following chart which clearly discloses that the improved method of treating metal powders as set forth herein provides a protective coating for metal powders which is far superior in the essential characteristics of preventing oxidation thereof, than those disclosed by prior art methods.

Percent weight increase of dried powder after exposure at 71° C., 95% relative humidity for indicated period

| Treatment                                | 12 Days' Exposure | 24 Days' Exposure |
|------------------------------------------|-------------------|-------------------|
|                                          | Percent           | Percent           |
| None.....                                | 3.25              | 5.24              |
| Dichromate only.....                     | .88               | 1.61              |
| Stearic Acid only.....                   | 1.21              | 3.75              |
| Dichromate followed by Stearic Acid..... | .10               | .29               |

After a careful study of the foregoing chart it will be apparent that the untreated metal powder deteriorated a considerable amount during the exposure time of 12 and 24 days and that the powder treated with either dichromate or stearic acid alone also showed considerable deterioration due to oxidation over such period of time. While on the other hand, the powder treated in the manner as heretofore set forth, first with dichromate followed by stearic acid treatment, deteriorated comparatively little over the same period of time as compared to the untreated powder, dichromate, or stearic acid treated powders.

It is probable that the acid ends of the stearic acid molecules are adsorbed by the film on the metal resulting from the dichromate treatment; leaving the aliphatic, hydrophobic ends of the molecules turned outward and thus providing the powder with a water repellent coating. It has been found that when the surfaces of the dichromate treated metal powder are covered with the stearic acid molecules, the attraction of additional molecules thereto ceases and thus after the powder has been stirred in a stearic acid solution for a sufficient period of time the surface thereof is covered therewith whereupon no further stearic acid will adhere thereto. Furthermore, it has been found that repeated washings of the aforementioned treated powder such, for example, as approximately 200 washings with fresh solvent, have failed to remove the protective coating from the powder. However, a lesser number of wash treatments are sufficient to remove the excess stearic acid. For example, by 10 washings with fresh solvent, the excess stearic acid is substantially removed from the powder leaving the strongly adsorbed stearic acid on the dichromate treated metal powder thereby providing a thin and uniform protective coating of controlled thickness on the particle surfaces thereof, which will not affect subsequent use of the powder.

As an example of the process of this invention, powdered manganese is stirred in a 5% solution of potassium dichromate in water. The solution is maintained at a temperature of approximately 80° C. and the stirring continued for approximately 30 minutes. The metal powder is then removed from the solution by filtering and thereafter washed with distilled water and dried. The dry treated powder resulting from the preceding step is then stirred in a solution of stearic acid in carbon tetrachloride. Thereafter the powder is again filtered and washed with carbon tetrachloride to remove the excess stearic acid. If the intended use of the powder is such that the excess stearic acid is not objectionable the

last washing step may be omitted. The resulting powder having an absorbed mono-molecular layer of stearic acid is found to be stable and resistant to decomposition.

The above process may be carried out with powdered cobalt as well as with manganese and process may also be carried out by substituting sodium dichromate for the potassium dichromate of the above example.

The reproducibility of the coating will be clearly apparent after a study of the following chart on which is shown the results of tests of two samples of manganese treated first with a dichromate solution and then with a stearic acid solution, the so-treated samples thereafter being washed thoroughly with a fresh solvent solution the results of which are also shown on the chart. It will be noted that the carbon content of the powder increased considerably after the dichromate and stearic acid treatment.

| 20 | Manganese Lots | Percent Carbon After | Percent Carbon After              | Calculated                                     |
|----|----------------|----------------------|-----------------------------------|------------------------------------------------|
|    |                | Dichromate Treatment | Subsequent Stearic Acid Treatment | Percent Carbon Added by Stearic Acid Treatment |
| 25 | 2007           | .010                 | .034                              | .024                                           |
|    | 2008           | .007                 | .032                              | .025                                           |

The percentage of carbon added by the stearic acid treatment provides a measure of the stearic acid adsorbed on the surface of the metal powder.

30 Since the quantity of stearic acid added to the surface of a metal powder by the aforescribed treatment probably depends on the surface area of the powder, it would be expected that a uniform coating procedure would result in an equal addition of stearic acid to each 35 of two similar lots of manganese. The results of the carbon analyses in the table indicate equal amounts of carbon, and, therefore, equal amounts of stearic acid are added to samples of the two lots of manganese. The maximum stearic acid that can be added to either lot is given by the following equation, assuming that the stearic acid is present in a monomolecular film:

$$W = \frac{A_m M}{A_s N}$$

45  $W$  = gm. stearic acid adsorbed in complete monolayer on one grain of manganese—Lot 2007 or 2008

$A_m$  = 1985 cm.<sup>2</sup>/gm. surface area of Lot 2007 or 2008 manganese as determined by nitrogen absorption method

50  $M$  = 284.5 gm. grain molecular weight of stearic acid  
 $A_s$  =  $22 \times 10^{-16}$  cm.<sup>2</sup> cross sectional area of stearic acid molecule

55  $N$  = Avogadro's Number  $6.06 \times 10^{23}$  molecules/gm. mol.

$W = \frac{1985 \times 284.5}{22 \times 10^{-16} \times 6.06 \times 10^{23}} = 424 \times 10^{-6}$  gram stearic acid absorbed in complete monolayer on one gram of Lot 2007 or 2008 manganese

60 The stearic acid actually adsorbed in one gram of manganese powder can be calculated from the carbon analyses of the coated powder by the following formula:

$$W_{st} = W_{c2} - W_{c1} \times \frac{Mst}{Mc}$$

65  $W_{st}$  = grams stearic acid adsorbed in one gram manganese  
 $W_{c2}$  = .00034 gm. carbon per gram of manganese after adsorption of stearic acid

$W_{c1}$  = .00010 gm. carbon per gram of manganese before adsorption of stearic acid

$Mst$  = 284.5 gm. gram molecular weight of stearic acid  
 $Mc$  = 216 gm. weight of carbon in one mol. of stearic acid

70  $W_{st} = .00025 \times \frac{284.5}{216} = 329 \times 10^{-6}$  grams of stearic acid adsorbed in one gram of hot 2007 manganese

75 Although these results indicate that there may not be sufficient stearic acid adsorbed in the manganese to cover

it completely with a monomolecular layer, there is certainly not sufficient stearic acid to cover the manganese with more than a monomolecular layer. Actually, the experimental error may be large enough to account for the fact that there does not appear to be sufficient stearic acid to cover the manganese completely.

From the foregoing, it will be apparent that a new and improved protective surface coating for metal powders has been provided which is far superior in deterioration-resistance characteristics than any of the coatings heretofore employed. Furthermore, from the foregoing it will be understood that a thin and uniform water repellent material of controlled thickness is applied to the particles of the metal powder, such coating being sufficiently thin so as not to affect subsequent use of the powder, the coating also being reproducible so that the properties of the powder are reproducible and thus the powder is admirably suited for use in pyrotechnic mixtures. Whereas, a more stable fuel is provided for use in a pyrotechnic mixture which will not be readily affected by atmospheric conditions and thus assuring proper delay and uniform burning time of the mixture after being stored over a long period of time under adverse weather conditions.

Obviously many modifications and variations of the present invention are possible in the light of the above teachings. It is therefore to be understood that within the scope of the appended claims the invention may be practiced otherwise than as specifically described.

What is claimed as new and desired to be secured by Letters Patent of the United States is:

1. A metal fuel for use in pyrotechnic mixtures and the like comprising a metal powder selected from the group consisting of cobalt and manganese, said metal powder having an inner coating of the oxide of said metal formed by the reaction of said metal with a warm aqueous solution of a dichromate selected from the group

25

30

35

consisting of sodium dichromate and potassium dichromate, and said metal powder having an outer coating formed by the reaction of said inner coating with a solution of stearic acid.

5. A metal fuel for use in pyrotechnic mixtures and the like comprising a finely divided metal selected from the group consisting of cobalt and manganese, said finely divided metal having an inner coating formed by the reaction of the metal with a warm aqueous solution of a dichromate selected from the group consisting of sodium dichromate and potassium dichromate, and said finely divided metal having an outer coating formed by the reaction of said inner coating with stearic acid.

10. 2. A metal fuel for use in pyrotechnic mixtures and the like comprising a finely divided metal selected from the group consisting of cobalt and manganese, said finely divided metal having an inner coating formed by the reaction of the metal with a warm aqueous solution of a dichromate selected from the group consisting of sodium dichromate and potassium dichromate, and said finely divided metal having an outer coating formed by the reaction of said inner coating with stearic acid.

15. 3. The method of providing pyrotechnic metal powders, such as cobalt, manganese and the like, with a protective water repellent coating, comprising immersing the metal powder in an aqueous solution containing about 5% of a dichromate selected from the group consisting of sodium dichromate and potassium dichromate at a temperature of from about 70° C. to about 95° C. for a period of about 30 minutes, drying said powder, and subsequently immersing said powder in a solution of stearic acid in an organic solvent.

15

20

25

#### References Cited in the file of this patent

##### UNITED STATES PATENTS

|           |                 |               |
|-----------|-----------------|---------------|
| 639,867   | Rosenberg       | Dec. 26, 1899 |
| 1,869,041 | Bengston        | July 26, 1932 |
| 2,206,064 | Thompson et al. | July 2, 1940  |
| 2,279,252 | Slunder         | Apr. 7, 1942  |
| 2,454,799 | Hart et al.     | Nov. 30, 1948 |

##### FOREIGN PATENTS

|         |               |               |
|---------|---------------|---------------|
| 218,619 | Great Britain | 1925          |
| 518,966 | Great Britain | Mar. 13, 1940 |
| 579,165 | Great Britain | July 25, 1946 |